

Nov. 9, 1943.

R. C. AMIDON

2,333,630

COMPOSITE FABRIC AND METHOD OF PRODUCING SAME

Filed Feb. 19, 1941

Fig. 1.



Fig. 2.



Fig. 3.



Fig. 4.



Inventor

Roy C. Amidon

By Albert E. Dietrich

Attorney

## UNITED STATES PATENT OFFICE

2,333,630

COMPOSITE FABRIC AND METHOD OF  
PRODUCING SAMERoy C. Amidon, St. Johnsville, N. Y., assignor to  
Vanity Fair Mills, Inc., a corporation of Penn-  
sylvania

Application February 19, 1941, Serial No. 379,687

21 Claims. (Cl. 28—73)

My invention relates to the textile art and, more particularly, to that branch of the art which has to do with the production of a fabric consisting of a base sheet combined with a knit fabric, such, for instance, as that disclosed in my Letters Patent No. 2,136,367 of November 15, 1938.

Primarily the present invention has for an object to provide a fabric of the character stated which may readily be embossed and which will retain its embossed appearance under all normal conditions of use.

Further, it is an object to provide a composite fabric and process of making the same, in which the base sheet through which the knitting takes place may not only be more or less vulcanized but which will be entirely enclosed by the knitting.

Further, the invention has for an object to produce a textile fabric which can be given the appearance of grained or embossed leather and which may be given an infinite number of surface designs.

Further, it is an object to provide a waterproof or water repelling fabric embodying the non-stretching characteristics of woven fabric with the ornamental appearances of knit fabric.

Other objects will in part be obvious and in part be pointed out hereinafter.

To the attainment of the aforesaid objects and ends the invention still further resides in the novel details of construction, combination and arrangement of parts, all of which will be first fully described in the following detailed description, and then be particularly pointed out in the appended claims, reference being had to the accompanying drawing, in which:

Figs. 1 to 4 are diagrammatic sectional views of different embodiments of the invention.

In carrying out my invention I may take a base sheet preferably composed of a suitable vulcanizable material such, for instance, as a sheet of partially vulcanized latex, or I may take a textile fabric saturated with latex, or other suitable material that can be vulcanized or stabilized by any suitable method, and knit through such base sheet according to the teachings disclosed in my Letters Patent No. 2,136,368 of November 15, 1938.

The knit fabric is then air or heat treated to vulcanize or set the base sheet material.

If the fabric is to be embossed, the vulcanization may take place at the same time as the embossing, by using heated embossing rollers, presses or molds.

As a further development of my process and product, after the base sheet has been passed through the knitting machine and before com-

plete vulcanization occurs, the knit fabric may be fulled or felted and the fabric then placed in a vulcanizing mold or press or passed between vulcanizing rollers, thereby anchoring down the surface threads so that the fulled or felted appearance of the fabric will be maintained indefinitely.

As a further development of my process, the article after completion of the knitting act may be passed through suitable dyeing apparatus before placing it in the final vulcanizing mold or press or passing it through the final vulcanizing rollers.

In carrying out my invention I may proceed as follows:

15 A sheet of woven fabric is passed through a bath of latex or may be sprayed with latex until the fabric becomes saturated (more or less) with the latex. The sheet is then passed over a vacuum or suction device to remove excess latex, and open the pores between the threads of the fabric; the latex-treated fabric is then passed through clay dust or other suitable material to dry the exposed latex on the threads; the base fabric is thereafter passed through the knitting machine (see my Letters Patent No. 2,136,368 aforesaid) and the two faces of the base fabric are thereby covered with the knit material; the latexed base sheet which the knit threads now cover may be further vulcanized to the extent desired by air or heat treatment, or in any other suitable way. When the fabric is to be an embossed fabric, this latter vulcanization step may be made to occur simultaneously with the embossing act by using heated embossing molds, presses or rollers.

If the finish desired is a fulled or felted finish, the surface of the knitting is fulled or felted before completing the vulcanization. When an elastic fabric is desired, instead of employing a base sheet composed of woven fabric saturated with latex, I may use a sheet of semi-vulcanized material such as latex, i. e., a material which has been sufficiently set so that knitting needles will puncture it, and pass this sheet through the knitting machine. This knit latex-base-sheet may have its surface fulled, felted or matted before placing it in the vulcanizing press or mold, or passing it between vulcanizing rollers.

Instead of using latex as a vulcanizable material as herein referred to, other suitable substances may be employed.

The use of latex impregnated fabric, or a latex sheet as a base fabric, or a layer of woven fabric and a layer of latex together, as a base sheet,

produces a waterproof or water repellent fabric, (Figs. 1 to 3 inclusive).

Instead of latex, I may use, for the purpose of producing a waterproof or water repelling fabric, a base sheet of woven fabric waterproofed by any other suitable substance or composition or in any other suitable way, (Fig. 4).

This application is a continuation in part of my application Serial Number 291,259, filed August 21, 1939.

Having thus described the invention, it is thought that the complete process and product will be clear to those skilled in the art.

What I claim is:

1. The method of making composite fabric which comprises knitting through a base sheet containing vulcanizable material, and thereafter effecting the vulcanization of said material to the extent desired.

2. The method of making composite fabric which comprises knitting through a base sheet containing vulcanizable material, thereafter effecting the vulcanization of said material to the extent desired, and simultaneously embossing the composite fabric.

3. The method of making a composite fabric which consists in knitting through a base sheet containing vulcanizable substance; then matting, fulling or felting the surface of the fabric, and finally applying pressure to the surface to set the same and vulcanizing the vulcanizable material.

4. The method of making a composite fabric which consists in saturating a sheet of woven textile material with latex; removing excess latex from the sheet and opening the pores thereof; drying the exposed latex on the sheet; passing the sheet through a knitting machine to knit through the sheet and enclose the base sheet in the knitting.

5. The method of making a composite fabric which consists in saturating a sheet of woven textile material with latex; removing excess latex from the sheet and opening the pores thereof; drying the exposed latex on the sheet; passing the sheet through a knitting machine to knit through the sheet and enclose the base sheet in the knitting; and then completing the vulcanization of the latex.

6. The method of making a composite fabric which consists in saturating a sheet of woven textile material with latex; removing excess latex from the sheet and opening the pores thereof; drying the exposed latex on the sheet; passing the sheet through a knitting machine to knit through the sheet and enclose the base sheet in the knitting; and then placing the composite sheet in a vulcanizing press or mold to set the latex.

7. The method of making a composite fabric which consists in saturating a sheet of woven textile material with latex; removing excess latex from the sheet and opening the pores thereof; drying the exposed latex on the sheet; passing the sheet through a knitting machine to knit through the sheet and enclose the base sheet in the knitting; and then placing the composite sheet in a vulcanizing and embossing press or mold to set the latex and emboss the fabric.

8. The method of making a composite fabric which consists in saturating a sheet of woven textile material with latex; removing excess latex from the sheet and opening the pores thereof; drying the exposed latex on the sheet; passing the sheet through a knitting machine to knit through the sheet and enclose the base sheet in

the knitting; and then felting the surface of the fabric; and finally completing the vulcanization.

9. The process of producing a composite fabric which consists in passing a sheet of woven fabric through a bath of latex until it becomes saturated with the latex; removing excess latex from the sheet by suction and opening the pores between the threads of the sheet; passing the latex-treated sheet through a suitable drying medium to dry the exposed latex on the threads; then passing the sheet through a knitting machine and covering both faces of the sheet with knitting material; and finally completing the vulcanization of the latex to the extent desired.

10. The process of producing a composite fabric which consists in passing a sheet of woven fabric through a bath of latex until it becomes saturated with the latex; removing excess latex from the sheet by suction and opening the pores between the threads of the sheet; passing the latex-treated sheet through a suitable drying medium to dry the exposed latex on the threads; then passing the sheet through a knitting machine and covering both faces of the sheet with knitting material; passing the composite sheet through a dyeing bath; and finally completing the vulcanization of the latex to the extent desired.

11. The process of producing a composite fabric which consists in passing a sheet of woven fabric through a bath of latex until it becomes saturated with the latex; removing excess latex from the sheet by suction and opening the pores between the threads of the sheet; passing the latex-treated sheet through a suitable drying medium to dry the exposed latex on the threads; then passing the sheet through a knitting machine and covering both faces of the sheet with knitting material; passing the composite sheet through a dyeing bath; and then embossing the composite sheet and completing the vulcanization of the latex to the extent desired.

12. A composite fabric, comprising a base sheet composed of vulcanizable latex, and a fabric knit through and embedding the base sheet before final vulcanization.

13. A composite fabric, comprising a base sheet composed of vulcanizable latex, and a fabric knit through and embedding the base sheet before final vulcanization, said composite fabric being embossed.

14. A composite fabric comprising a base sheet of textile material impregnated with latex, and a fabric knit through said base sheet and covering both faces thereof, a surface of the composite fabric being embossed and the latex on vulcanizing serving to "fix" the embossing.

15. A composite fabric comprising a base sheet of textile material impregnated with vulcanizable latex, and a fabric knit through said base sheet and covering both faces thereof, the outer faces of the composite fabric being fulled.

16. A composite fabric comprising a base sheet of textile material impregnated with vulcanizable latex, and a fabric knit through said base sheet and covering both faces thereof, the outer faces of the composite fabric being felted.

17. A composite fabric comprising a base sheet of textile material impregnated with vulcanizable latex, and a fabric knit through said base sheet and covering both faces thereof, the fabric being knit to produce an ornamental surface.

18. A composite fabric comprising a base sheet of textile material impregnated with latex, and a fabric knit through said base sheet and cover-

ing both faces thereof, the fabric being embossed and the latex on vulcanization serving to "fix" the embossings.

19. A composite fabric comprising a vulcanizable waterproof base fabric and a fabric knit through the same.

20. A composite fabric comprising a base sheet composed of a layer of woven fabric and at least

one layer of vulcanizable latex, and a fabric knit through the same.

21. A composite fabric comprising a base sheet composed of a layer of woven fabric and at least one layer of vulcanizable material and a fabric knit through the same, the fabric being embossed and the vulcanizable material serving to fix the embossings.

ROY C. AMIDON.